

F. KEENAN.

Improvement in Coffins from Paper or other Pulps.

No. 123,781.

Patented Feb. 20, 1872.



Witnesses:

Chas. Nida.  
H. L. Wattenberg

Inventor:  
Franklin Keenan  
per G. M. Chapman.

Atty-

## UNITED STATES PATENT OFFICE.

FRANKLIN KEENAN, OF BROWNVILLE, NEW YORK.

## IMPROVEMENT IN COFFINS FROM PAPER OR OTHER PULP.

Specification forming part of Letters Patent No. 123,781, dated February 20, 1872.

*To all whom it may concern:*

Be it known that I, FRANKLIN KEENAN, of Brownville, in the county of Jefferson and State of New York, have invented a new and useful Improvement in Coffins; and that the following is a full and exact description of the same, reference being had to the accompanying drawing and to the letters of reference marked thereon making a part of this specification.

The object of this invention is to produce a coffin which shall be cheap, strong, light, and easily made. The invention consists in making the coffin of any suitable pulp, and then forming it in molds in the manner hereinafter described.

In the accompanying sheet of drawing, Figure 1 is a plan view of my invention, and Fig. 2 a side view, partly in section.

Similar letters of reference indicate like parts in the several figures.

A represents a coffin, which may be of any desirable shape and size, and it differs from coffins as ordinarily made, in that, instead of being constructed of wood or metal, it is made of a semi-fluid pulp. This pulp may be made from either paper, wood, leather, or any other material.

To construct my coffin, I first produce the pulpy substance in any of the well-known ways of making pulp; and, having previously prepared a suitable metallic mold, I charge the mold with the pulp, then, by a suitable follower, subject the pulp in the mold to a pressure which forces out the surplus moisture and forms the pulp into a compact mass. The mold

with the pulp therein is then inclosed in a cylinder or other suitable steam-tight vessel, and by admitting steam to said vessel it entirely surrounds the mold inside and out, and effectually dries the coffin, which may then be readily removed by taking the mold apart. The coffin is thus produced with the bottom sides and ends in one continuous compact body, the lid being formed separate from the body of the coffin; also, by pulp in molds, in a similar manner to that above described; after which the coffin may be smoothed with pumice, if desired, and suitably finished to represent various kinds of woods, or lacquered to represent metal.

It will be observed that the lid of my coffin has a molding or lip, which projects around and over the upper edge of the coffin, so that, while the projecting edge or lid furnishes a means of securing the lid to the coffin by passing screws through it into the coffin, it also furnishes a means of stiffening the sides of the coffin, thus preventing any liability of the sides bulging out from any cause whatever.

I do not wish to confine myself to thus forming the coffin of any particular kind of pulp, nor to any particular means of molding the pulp; but

What I do claim as new, and desire to secure by Letters Patent, is—

A coffin made from pulp in the manner and for the purposes hereinbefore described.

FRANKLIN KEENAN.

Witnesses:

H. L. WATTENBERG,  
G. M. PLYMPTON.